

Nov. 2, 1948.

S. F. W. WELFORD

2,452,705

PACKAGE OF PHOTOGRAPHIC LIGHT-SENSITIVE PAPERS

Filed Feb. 23, 1945



INVENTOR.

*Stanley Frederick William Welford*  
BY

*Lynn Barratt Morris*

ATTORNEY

## UNITED STATES PATENT OFFICE

2,452,705

## PACKAGE OF PHOTOGRAPHIC LIGHT-SENSITIVE PAPERS

Stanley Frederick William Welford, Ilford, England, assignor to Ilford Limited, Ilford, England, a British company

Application February 23, 1945, Serial No. 579,489  
In Great Britain March 3, 1944

1 Claim. (Cl. 95—8)

1

This invention relates to photographic materials and particularly to photographic printing papers and the like.

In British Patent No. 550,775 there is described a method of producing a photographic image wherein a sensitive silver salt paper, coated on its sensitive surface with a layer of a binder which is insoluble in plain water but soluble in alkali solutions, is exposed with the sensitive surface in contact with a wet negative, and subsequently developed. When a paper so coated is placed in an alkaline developing solution, the alkali therein causes the coating to dissolve.

A number of specific binders are described in the said specification which may be used as the coatings in question. Among these are polyvinyl acid esters, especially of dibasic acids, such as polyvinyl acetate phthalate, esters of polybasic acids, and the compounds formed by condensing a terpene with an  $\alpha$ - $\beta$ -unsaturated polycarboxylic acid or acid anhydride such as maleic acid anhydride. Among the other materials listed as suitable are the alkyd resins, which are condensation products of polyhydric alcohols as, for example, glycols, glycerol, sugars and simple derivatives thereof, with polycarboxylic acids, for example citric, maleic, phthalic, succinic and tartric acids.

Another material which may be so employed is a polymerised methyl methacrylate resin which contains free carboxyl groups, described in U. S. application No. 581,564, filed March 7, 1945, now abandoned, corresponding to British application No. 1,965/44.

It has been found in practice that a difficulty arises in many cases, and particularly in the case where alkyd resin binders are employed, that there is a tendency for the resin, on keeping, to become less soluble in alkali, thus increasing the time necessary for development, or even rendering the material useless. This "insolubilisation" is accelerated under tropical conditions.

According to the present invention, the insolubilisation of the binder resin, and especially of alkyd resins used for this purpose, is prevented or retarded by packing the light-sensitive elements in such a way that the only layers in contact with the binder resin coatings are either similar binder resin coatings or are protein layers.

Normally the resin binder coatings are directly superimposed on gelatino silver halide emulsion layers, though there may be a water-permeable intermediate gelatin layer. Thus the object of this invention may be achieved by packing the light-sensitive elements in pairs with the resin

coatings face to face. Thus a number of sheets of the light-sensitive element may be disposed in a pile, each successive pair having their binder resin surfaces in contact.

5 Alternatively the rear face (back) of the element may also be provided with a coating of the binder resin in which case the desired result is achieved whichever way the elements are packed.

However, these methods are not always entirely 10 satisfactory since, although they prevent or retard the insolubilisation of the resin, there is a tendency for the resin layers to stick together, especially in the case of large packets of the elements, where the weight of the elements is 15 considerable.

A preferred method, therefore, is to provide the light-sensitive element with a protein backing layer. Thus the element may consist of a paper support coated on one side with a gelatino silver halide emulsion layer supercoated with a resin binder layer which is water-insoluble but alkali-soluble, and coated on the other side with a plain gelatin layer. Such elements, when packed face to back, fulfil the object of this invention, i. e. the 20 resin binder layer on the face of one element is in contact only with the protein layer on the binder face of the next adjacent element, and there is very little tendency for the resin layer to become insoluble or for the elements to stick 25 together.

A pack of the elements just described is shown 30 in perspective in the accompanying drawing wherein a paper base 1 is provided on its upper surface with a gelatino silver halide emulsion 35 layer 2. A layer 3 composed of an alkyd resin which is water-insoluble but alkali-soluble is disposed on the emulsion layer. The rear surface of the base is provided with a gelatin layer 4. The latter layer of each successive element in the pack 40 is placed in contact with the resin layer 3 of the next successive element.

According to a further feature of this invention, therefore, a photographic element suitable 45 for printing from wet negatives comprises a support, e. g. of paper, coated on one side with a gelatino silver halide emulsion layer super-coated with a layer of a binder which is water-insoluble but alkali-soluble, and coated on the other side with a protein, e. g. gelatin, layer.

50 A convenient method of securing the protein backing coat is to apply to the back of the element a 4% aqueous solution of gelatin. Other protein layers may, however, be employed, e. g. casein or zein.

55 This invention is of primary importance where

the binder employed is an alkyd resin, e. g. a resin such as the product sold commercially under the trade name Paralac 1101 but may be employed in connection with other resins used for the same purpose. The resin binder may contain a plasticizer if desired, e. g. tricresyl phosphate.

The methods of avoiding insolubilisation according to the present invention present the advantage of economy over such expedients as the use of interleaving sheets of wax paper, which also functions, and avoids the difficulties to which waxed paper tends to give rise under tropical conditions.

The following examples illustrate the invention:

*Example 1*

A wet-printing photographic paper consisting of a paper base coated on one side first with a plain gelatin layer, then with a layer of silver halide gelatin emulsion, and then with a layer of the alkyd resin sold under the name Paralac 1101, was coated on the other side with a solution consisting of:

|               |        |       |
|---------------|--------|-------|
| Casein        | grams  | 100   |
| Slaked lime   | do     | 18    |
| Caustic soda  | do     | 11    |
| Water to make | liters | 1 1/2 |

The solution was filtered through muslin before use. When dry this coating felt slightly rough to the touch.

*Example 2*

A wet-printing paper of the character described in Example 1 was coated on its rear face with a 4% aqueous solution of gelatin containing small proportions of chrome alum and formaldehyde as hardening agents.

*Example 3*

A printing paper consisting of a paper base coated on one side with a plain gelatin layer and then with a silver halide gelatin emulsion layer was coated on both sides with a 10% solution in acetone of the resin sold under the name Paralac 1101 containing 30-40 cc. per gallon of tricresyl phosphate.

The products of all these examples showed an improvement over the corresponding products having no coating on the rear surface of the paper base, in that the tendency of the resin coating to become insoluble in alkali was much reduced. The products of Examples 1 and 2 are preferably packed face to back and thus packed show a much reduced tendency to sticking, while those of Example 3 may be packed either face to back or face to face.

What I claim is:

A package of light-sensitive elements each element comprising a paper support carrying on one side thereof a gelatino silver halide emulsion layer and a superimposed layer of an alkyd resin which is water-insoluble but alkali-soluble and carrying on the other side thereof a layer of gelatin, the said elements being packed in the package face to back.

20

STANLEY FREDERICK  
WILLIAM WELFORD.

REFERENCES CITED

25 The following references are of record in the file of this patent:

UNITED STATES PATENTS

| Number       | Name          | Date           |
|--------------|---------------|----------------|
| 30 253,354   | Eastman       | Feb. 7, 1882   |
|              | 778,740       | Dec. 27, 1904  |
| 35 1,180,415 | Nasief et al. | Apr. 25, 1916  |
|              | 1,261,748     | McCurdy        |
| 35 1,342,590 | Lovejoy       | Apr. 2, 1918   |
| 35 2,090,016 | Young et al.  | June 8, 1920   |
|              | 2,173,480     | Young et al.   |
| 35 2,372,935 | Jung          | Aug. 17, 1937  |
|              | 2,373,289     | Challis        |
| 40 2,373,732 | Brown         | Sept. 19, 1939 |
|              | 2,391,181     | Wolfsen        |
|              |               | Apr. 3, 1945   |
|              |               | Apr. 10, 1945  |
|              |               | Apr. 17, 1945  |
|              |               | Dec. 18, 1945  |

FOREIGN PATENTS

| Number     | Country       | Date          |
|------------|---------------|---------------|
| 45 424,976 | Great Britain | Mar. 6, 1935  |
|            | 482,204       | Mar. 24, 1938 |
|            | 550,775       | Great Britain |
|            |               | Jan. 25, 1943 |